

United States Patent  
Martini

[15] 3,671,408  
[45] June 20, 1972

[54] RHODIUM-PLATINUM PLATING BATH  
AND PROCESS

[72] Inventor: Albert Michael Martini, Florham Park, N.J.  
[73] Assignee: Sel-Rex Corporation, Nutley, N.J.  
[22] Filed: May 25, 1971  
[21] Appl. No.: 146,808

[52] U.S. Cl.....204/43  
[51] Int. Cl.....C23b 5/32  
[58] Field of Search.....204/43, 47, 123

[56] References Cited

UNITED STATES PATENTS  
2,984,604 5/1961 Duva et al.....204/47

3,515,651 6/1970 Ohkubo.....204/43  
3,528,895 9/1970 Simonian.....204/47 X

OTHER PUBLICATIONS

Abner Brenner, "Electrodeposition of Alloys," Vol. II, pp. 544-545, (1963).

Primary Examiner—G. L. Kaplan  
Attorney—Samuel Kriegel

[57] ABSTRACT

An electrolyte and process for electrodepositing a low stress and mirror bright rhodium-platinum alloy. The electrolyte comprises an aqueous solution of rhodium sulfate, platinum as P salt and sulfamic acid.

13 Claims, No Drawings

## RHODIUM-PLATINUM PLATING BATH AND PROCESS

## BACKGROUND OF THE INVENTION

Electrodeposited rhodium is used for a decorative coating and as a contact base metal because of its extreme hardness and resistance to corrosion and to wear. Rhodium plating is particularly useful as a protective coating for silverware, hollow ware, jewelry and for electronic products. Such deposits, however, tend to be brittle, especially thick deposits.

Electrodeposited platinum has not been as popular as rhodium in the jewelry and decorative field because its color is darker than rhodium or silver and it tends to darken further with time. There would be a great interest in the above areas for obtaining bright low stress deposits of rhodium, platinum or mutual alloys of the two.

It is an object of this invention to provide a novel rhodium-platinum plating bath which produces brighter electrodeposits than can be obtained from a bath of either metal alone.

It is a further object of this invention to provide a novel process for obtaining brighter rhodium-platinum electrodeposits.

It is a more specific object of this invention to provide a novel plating bath which produces a ductile, low stress, mirror bright rhodium-platinum deposit.

It is another object of this invention to obtain an electroplated article having a ductile, low stress, mirror bright rhodium-platinum deposit.

Other objects and advantages of this invention become apparent from the following description.

## SUMMARY OF THE INVENTION

Although  $\text{Pt}(\text{NH}_3)_2(\text{NO}_2)_2$  — sulfamic acid baths yield dull electrodeposits and rhodium sulfate — sulfuric acid baths yield satin or semi-bright electrodeposits, it has unexpectedly been found that when an aqueous solution of  $\text{Pt}(\text{NH}_3)_2(\text{NO}_2)_2$ , (also referred to as platinum P salt) rhodium sulfate, and sulfamic acid is used for electroplating, a rhodium-platinum deposit of improved brightness is obtained. In particular, when rhodium is the predominant metal in the bath the deposit obtained is mirror bright.

## DETAILED DESCRIPTION

In practicing the present invention rhodium sulfate, platinum P salt, and sulfamic acid are generally mixed with sufficient water to obtain the following approximate concentrations:

|                                     |                                |
|-------------------------------------|--------------------------------|
| Rhodium metal (as the sulfate)      | 0.1—15g/l                      |
| Platinum metal (as platinum P salt) | 0.04—24.0g/l                   |
| Sulfamic acid                       | 20g/l—saturation concentration |

Preferably the rhodium metal concentration ranges from about 0.5 to 12 g/l, most preferably from about 2 to 10 g/l. Preferably, the platinum metal varies from about 0.07 to 12 g/l, most preferably from about 0.1 to 10 g/l. The sulfamic acid concentration preferably varies from 30 g/l to saturation concentration, most preferably from 50 to 100 g/l.

A high rhodium bath is used for electrodepositing a predominantly rhodium containing alloy. In this high rhodium bath, the rhodium metal concentration generally ranges from about 1 to 12 g/l, preferably from about 2 to 7 g/l; the platinum metal concentration varies from about 0.04 to 1.2 g/l, preferably from about 0.1 to 0.7 g/l; and the sulfamic acid concentration varies from about 30 g/l to saturation concentration, preferably 50 to 100 g/l. The rhodium concentrations for the high rhodium bath can be further broken down according to the thickness of the deposit desired. For deposits of up to about 2 microinches thickness it is preferred that the rhodium content of the bath be 1 to 2 g/l; for deposits of 2 to 10 microinches, the rhodium content preferably is 2 to 5 g/l; and for deposits greater than 10 microinches, the rhodium content preferably is 2 to 10 g/l. The platinum content for each range of thickness varies proportionately with the rhodium content.

A high platinum bath is used for electrodepositing a predominantly platinum containing alloy. In this high platinum bath, the platinum metal concentration varies from about 2 to 24 g/l, preferably from about 5 to 12 g/l; the rhodium metal concentration varies from about 0.10 to 5 g/l, preferably from about 0.2 to 2 g/l; and the sulfamic acid concentration varies from about 30 to saturation, preferably from about 50 to 100 g/l.

In all the above baths, the limits of current density can usually be improved by the addition of concentrated sulfuric acid generally up to about 100 ml/l of solution, preferably from 1 to 50 ml/l of solution.

The plating solution of this invention can be used to coat any substrate that is capable of receiving an electrodeposit, particularly such basis metals as copper, brass, nickel, mild steel, silver and the like. Because the acid bath of this invention might cause dissolution of the basis metal thereby contaminating the bath, it is preferred that the basis metal be protected, eg. by flash coating with palladium, palladium-gold, or preferably gold, so as to inhibit attack on the basis metal. In the case where the basis metal contains iron, it is preferred that the basis metal first be preplated with, for example, nickel, copper, or silver, prior to flash coating. The rhodium-platinum alloy may be deposited from the plating bath, at a temperature of about 60° to 180° F., by passing a current at a current density of about 5 to 40 ASF through the bath to a cathode immersed therein. Preferably the current density is about 10 to 30 ASF and the temperature about 80° to 130° F. The lower temperatures are generally used for flash deposits and the higher temperatures for heavier deposits and for high platinum deposits.

The deposit obtained using the high platinum bath contains from about 90 to 99 percent platinum, preferably from about 93 to 98 percent by weight. The high rhodium bath yields a low stress, predominantly rhodium containing deposit which is mirror bright, ductile, and contains from about 90 to 99.5 percent rhodium, preferably from about 93 to 99 percent rhodium, most preferably from 96 to 98.5 percent rhodium by weight, and from about 0.5 to 10 percent platinum, preferably from about 1.0 to 7 percent platinum, most preferably from about 1.5 to 4.0 percent platinum by weight.

The deposits obtained by the process of this invention range from flash coatings, eg. 2 microinches, up to thick coatings of 200 microinches or more. Preferably this process is used to obtain low stress deposits of 50 to 150 microinches.

The addition of trace quantities of lead to the high rhodium bath of this invention increases the life of the bath with respect to mirror bright deposits. Generally, up to 10 mg. of lead metal is added per liter of bath, preferably from 2 to 6 mg/liter. The lead is added as a water soluble salt, preferably as lead nitrate.

The high rhodium bath is particularly useful for the plating of coins, jewelry, hollow ware, tableware, and the like, giving a mirror bright finish which greatly adds to their appearance. The high rhodium bath is especially useful for plating silver articles, preferably those containing greater than 90 weight percent silver, in that the deposit inhibits tarnishing of the silver, probably because of the non-porous nature of the deposit. In plating silver articles with the high rhodium bath, it is preferred that the article first be given a flash coating of gold.

The invention may be further illustrated by the following examples:

## EXAMPLE 1

|                          |                           |
|--------------------------|---------------------------|
| Bath Volume - One Liter: |                           |
| Rhodium metal            | 2gms (as the sulfate)     |
| Platinum metal           | 0.05 (as platinum P salt) |
| Sulfamic acid            | 30gms.                    |
| Sulfuric acid            | 5ml. concentrated         |
| Cathode efficiency:      |                           |
| with agitation           | 12mg/Amp.min.             |
| without agitation        | 6—9mg/Amp.min.            |

Test Panels are brass-gold struck

Mirror bright deposits are obtained at 15 to 20 ASF and 110° to 120° F without agitation.

With agitation at 15 to 20 ASF and 110° to 120° F, full bright deposits are obtained except for slight haze on higher current density edges of panels.

Platinum metal increased to 0.12 g/l resulting in mirror bright deposits with agitation, eliminating the slight haze at 15 ASF. Slight haze still occurs however, at 20 ASF on edges of test panel.

Test panel is plated to 100 microinches, with agitation, and analysis shows that deposit contains 2 to 5 percent Pt. and is low stress.

Various items are plated in the above baths, including nail clippers, tie-tacks, rings, and pickle fork with similar results.

#### EXAMPLE 2

| Bath:                 | Rh metal      | 2gms/l (as the sulfate)  |
|-----------------------|---------------|--------------------------|
|                       | Pt metal      | 0.2gms/l (as the P salt) |
|                       | Sulfamic acid | 90gms/l                  |
| Operating conditions: |               |                          |
| Temperature           | 115-118°F     |                          |
| No agitation          |               |                          |
| C.D.                  | 15ASF max     |                          |

Test panels: Bright nickel plated brass with gold strike.

Plating results:

Test panels are plated mirror bright (15ASF) with a finish approaching the color of a highly buffed silver piece. — 0.5 to 5 minutes.

Thickness: Flash to 10 microinches.

Other items plated mirror bright with the above bath are: nail clippers - - - - bright nickel + gold flash coins (silver) - - - palladium gold flash and gold flash candle labrum- - - - total area - - 2 square feet. - - bright nickel plated+ gold flash.

#### EXAMPLE 3

| Bath: | Rhodium metal  | 5gms/l    |
|-------|----------------|-----------|
|       | Platinum metal | 0.5 gms/l |
|       | Sulfamic acid  | 90 gms/l  |
|       | Sulfuric acid  | 5 ml/l    |

Items plated with the above bath:

- Brass watch bezels are plated at 118° to 122° F. and 20 ASF for 20 to 42 minutes. Mirror bright, silver colored deposits are obtained having thicknesses of 100 to 200 microinches.
- 2 to 14K gold rings are plated at 115° F. and 20 ASF for 5 minutes, without agitation. Deposits obtained are 10 to 15 microinches and mirror bright, and have a silver color.
- Test panel of nickel plated brass with gold flash is plated at 110° to 115° F. and 20ASF, with agitation for 10 minutes. Deposit is 50 to 70 microinches, mirror bright and low stress, and has a silver color.

#### EXAMPLE 4

| Bath | Rhodium metal   | 2 gms/liter<br>(as the sulfate)  |
|------|-----------------|----------------------------------|
|      | Platinum metal  | 0.2 gms/liter<br>(as the P salt) |
|      | Sulfamic acid   | 90 gms/liter                     |
|      | Sulfuric acid   | 5 ml/liter                       |
|      | Distilled water | (conc. $H_2SO_4$ )<br>to volume  |

- A test panel of nickel plated brass with gold strike is plated at 110° to 115° F. and 20ASF for 2 minutes without agitation. A 2 microinch mirror bright deposit is obtained having a silver color.
- A test panel of nickel plated brass with gold strike is plated at 115° F. and 20 ASF for 10 minutes with agitation. A mirror bright deposit of 40 to 50 microinches is obtained.
- Sterling silver coins are gold struck and then plated for 2 minutes at 110° to 114° F. and 20 ASF with no agitation. Mirror bright deposits of 3 to 5 microinches are obtained.

#### EXAMPLE 5

| 15 | Bath            | Rhodium metal                   | 2 gms/liter<br>(as the sulfate) |
|----|-----------------|---------------------------------|---------------------------------|
| 20 | Platinum metal  | 12 gms/liter<br>(as the P salt) |                                 |
|    | Sulfamic acid   | 100 gms/liter                   |                                 |
|    | Distilled water | to volume                       |                                 |

25 A test panel of nickel plated brass with gold strike is plated at 150° to 175° F. and 20 ASF for 17 minutes with agitation. A 100 microinch semi-mirror bright deposit is obtained.

I claim:

1. An electroplating bath for depositing rhodium-platinum alloy therefrom comprising an aqueous solution of:

|                                |                                  |
|--------------------------------|----------------------------------|
| Rhodium metal (as the sulfate) | 0.1 to 15g/l                     |
| Platinum metal (as P salt)     | 0.04 to 24g/l                    |
| Sulfamic acid                  | 20g/l - saturation concentration |

30 2. The bath of claim 1 comprising an aqueous solution of:

|                                |                                  |
|--------------------------------|----------------------------------|
| Rhodium metal (as the sulfate) | 0.5 to 12g/l                     |
| Platinum metal (as P salt)     | 0.07 to 12g/l                    |
| Sulfamic acid                  | 30g/l - saturation concentration |

35 3. The bath of claim 2 additionally containing up to about 100 ml/l concentrated sulfuric acid per liter of solution.

45 4. An electroplating bath for depositing a predominantly rhodium containing alloy comprising an aqueous solution of:

|                                |                                   |
|--------------------------------|-----------------------------------|
| Rhodium metal (as the sulfate) | 1 to 12g/l                        |
| Platinum metal (as P salt)     | 0.04 to 1.2g/l                    |
| Sulfamic acid                  | 30 g/l - saturation concentration |

50 5. The bath of claim 4 comprising an aqueous solution of:

|                                |                                   |
|--------------------------------|-----------------------------------|
| Rhodium metal (as the sulfate) | 2 to 7g/l                         |
| Platinum metal (as P salt)     | 0.1 to 0.7g/l                     |
| Sulfamic acid                  | 30 g/l - saturation concentration |

55 6. The bath of claim 5 wherein the sulfamic acid concentration is 50 to 100 g/l.

7. The bath of claim 6 additionally containing up to about 100 ml/l of concentrated sulfuric acid per liter of solution.

8. The bath of claim 6 which additionally contains trace amounts of lead in solution.

65 9. The bath of claim 5 additionally containing up to about 100 ml/l of concentrated sulfuric acid per liter of solution.

10. A process of electroplating rhodium-platinum alloy comprising electrodepositing the rhodium and platinum upon a basis metal from the aqueous bath of claim 1.

70 11. A process for electroplating a predominantly rhodium containing alloy comprising electrodepositing rhodium and platinum upon a basis metal from the bath of claim 4.

12. A process for electroplating a predominantly rhodium containing alloy comprising electrodepositing rhodium and platinum upon a basis metal from the bath of claim 5.

13. A process for electroplating a predominantly rhodium containing alloy comprising electrodepositing rhodium and platinum upon a basis metal from the bath of claim 8.

11. A process for electroplating a predominantly rhodium containing alloy comprising electrodepositing rhodium and 5 platinum upon a basis metal from the bath of claim 4.

\* \* \* \* \*

10

15

20

25

30

35

40

45

50

55

60

65

70

75